

## UNITED STATES PATENT OFFICE.

FRED PALMER AND FRANK PALMER, OF SPOKANE, WASHINGTON.

## PROCESS FOR TREATMENT OF METALS.

No Drawing.

Application filed April 29, 1921. Serial No. 465,494.

To all whom it may concern:

Be it known that we, FRED PALMER and FRANK PALMER, citizens of the United States, residing at Spokane, in the county of Spokane and State of Washington, have invented certain new and useful Improvements in Processes for Treatment of Metals, of which the following is a specification.

This invention relates to an improved process for refining metal.

The primary object of the invention is the provision of a special liquid bath or solution, for quenching of heating metals, as a means of refinement of said metals.

A further object of the invention is the provision of a liquid bath made from the subsequently described formula, and adapted for carburizing metals when quenched therein.

A further object of the invention is the provision of a liquid solution of the above described character specifically adapted to simultaneously harden, toughen, and carburize mild steels, by their immersion therein, when heated to a critical temperature.

Other objects and advantages will be apparent during the course of the following detailed description.

The specific proportions of ingredients in the improved metal refining bath are as follows:

|                                                  |          |
|--------------------------------------------------|----------|
| Sodium sulphate ( $Na_2SO_4$ )                   | 2 ounces |
| Sodium chloride $NaCl$                           | 8 ounces |
| Potassium ferrocyanide ( $K_4Fe(CN)_6 + 3H_2O$ ) | 2 ounces |
| Water ( $H_2O$ )                                 | 1 gallon |

The bath or solution is preferably used in connection with mild steels of varying carbon content, and which may have as high a carbon content as 1.1% or 1.2%. A high degree of refinement and carburization of this grade of metal has resulted from the precise use of the above proportioned formula, although the same may be varied slightly to suit the analyses of the various ingredients; as where an alkali water is used, the sodium sulphate can be decreased proportionately.

The mild steel or other metal is first slowly heated throughout until it reaches its critical temperature, which takes place at a color glow of bright cherry red, ranging from  $1380^\circ$  to  $1460^\circ$  Fahrenheit. At this temperature the grain of the steel is refined until it possesses the finest structure which it is capable of assuming. After the metal is heated evenly throughout, it is taken from the furnace at its critical temperature, and suddenly quenched in a cold bath of the above set forth ingredients and proportions. The bath preferably ranges from  $40^\circ$  to  $85^\circ$  Fahrenheit; and is of sufficient quantity to evenly cool the metal throughout, without itself absorbing too much heat from the metal.

By reason of its sudden immersion in this bath, the refined grain of the mild steel is retained, the immersion, hardening, toughening and carburizing the same. The toughening, hardening, and carburizing are effected simultaneously by chemical action of the solution upon the heated steel, and which steel requires no subsequent tempering to lessen brittleness, or relieve strains therein. This process of refining is in direct contrast to the ordinary method of hardening metals, where a bath of ordinary water is used for immersion of the heated metal, and which while resulting in a hardening of the metal results in still more rapidly increasing brittleness. Treatment of metals under this ordinary process requires subsequent tempering in order to toughen and relieve the metal of strain.

As before stated, the bath works best upon mild steels of various carbon contents. In an analysis of the physical properties before and after treatment, the ultimate tensile strength was shown by a Reihle machine to have increased from 64,000 pounds per square inch to 91,200 pounds per square inch; while the percentage of carbon as demonstrated by Prof. Arnold's chromic acid test was increased from 1.1% to 2.058%. Thus the special bath treatment of mild steel will produce a straight carbon tool steel of exceptional physical properties.

Various alterations in the process may be made without departing from the spirit of the invention, or the scope of the claims.

I claim:

- 5 1. A liquid bath for treatment of metals comprising sodium sulphate, salt, potassium ferrocyanide, and water.
2. A liquid bath for treatment of metals comprising in proportion:
- 10 Sodium sulphate ( $\text{Na}_2\text{SO}_4$ ) ----- 2 ounces  
Sodium chloride ( $\text{NaCl}$ ) ----- 8 ounces  
Potassium ferrocyanide  
    ( $\text{K}_4\text{Fe}(\text{CN})_6 + 3\text{H}_2\text{O}$ ) ----- 2 ounces  
Water ( $\text{H}_2\text{O}$ ) ----- 1 gallon
- 15 3. The method of hardening and tempering metals which consists in the quenching of a metal in a liquid bath composed of sodium sulphate, salt, potassium ferrocyanide and water.
- 20 4. The method of hardening and tempering metals which consists in heating a metal to the critical temperature and quenching the same in a liquid bath of sodium sulphate, salt, potassium ferrocyanide and water.
- 25 5. The method of hardening and tempering metals which consists in heating a metal to its critical temperature, and then quenching in a liquid bath comprising in proportion:
- 30 Sodium sulphate ( $\text{Na}_2\text{SO}_4$ ) ----- 2 ounces  
Sodium chloride ( $\text{NaCl}$ ) ----- 8 ounces  
Potassium ferrocyanide  
    ( $\text{K}_4\text{Fe}(\text{CN})_6 + 3\text{H}_2\text{O}$ ) ----- 2 ounces  
Water ( $\text{H}_2\text{O}$ ) ----- 1 gallon
- 35 6. The method of carburizing metal which consists of heating said metal to a critical temperature and quenching said metal in bath of sodium sulphate, salt, potassium ferrocyanide and water.
- 40 7. The method of carburizing metal, which consists of heating said metal to its critical temperature and quenching in a liquid bath comprising in proportion:
- 45 Sodium sulphate ( $\text{Na}_2\text{SO}_4$ ) ----- 2 ounces  
Sodium chloride ( $\text{NaCl}$ ) ----- 8 ounces  
Potassium ferrocyanide  
    ( $\text{K}_4\text{Fe}(\text{CN})_6 + 3\text{H}_2\text{O}$ ) ----- 2 ounces  
Water ( $\text{H}_2\text{O}$ ) ----- 1 gallon
- 50 8. The method of producing a straight carbon steel, which consists in heating a mild

steel to its critical temperature, and quenching the same in a bath of sodium sulphate, salt, potassium ferrocyanide, and water.

9. The method of producing a straight carbon steel, which consists in heating a mild steel to its critical temperature and quenching the same in a liquid bath comprising in proportion:

|                                                                                              |          |    |
|----------------------------------------------------------------------------------------------|----------|----|
| Sodium sulphate ( $\text{Na}_2\text{SO}_4$ ) -----                                           | 2 ounces | 65 |
| Sodium chloride ( $\text{NaCl}$ ) -----                                                      | 8 ounces |    |
| Potassium ferrocyanide<br>( $\text{K}_4\text{Fe}(\text{CN})_6 + 3\text{H}_2\text{O}$ ) ----- | 2 ounces |    |
| Water ( $\text{H}_2\text{O}$ ) -----                                                         | 1 gallon |    |

10. The method of refining mild steels which consists in simultaneously hardening, toughening and carburizing said mild steel to produce a tool steel by heating said mild steel to its critical temperature and quenching in a liquid bath of sodium sulphate, salt, potassium ferrocyanide, and water.

11. The method of refining mild steels which consists in simultaneously hardening, toughening and carburizing said mild steel to produce a tool steel by heating said mild steel to its critical temperature and quenching in a liquid bath comprising in proportion:

|                                                                                              |          |    |
|----------------------------------------------------------------------------------------------|----------|----|
| Sodium sulphate ( $\text{Na}_2\text{SO}_4$ ) -----                                           | 2 ounces | 85 |
| Sodium chloride ( $\text{NaCl}$ ) -----                                                      | 8 ounces |    |
| Potassium ferrocyanide<br>( $\text{K}_4\text{Fe}(\text{CN})_6 + 3\text{H}_2\text{O}$ ) ----- | 2 ounces |    |
| Water ( $\text{H}_2\text{O}$ ) -----                                                         | 1 gallon |    |

12. The method of refining metals which consists in heating a metal to a bright cherry red color, and suddenly immersing the same in a cold bath of sodium sulphate, salt, potassium ferrocyanide and water.

13. The method of refining metals, which consists in heating a metal to a bright cherry red color, and suddenly immersing the same in a cold liquid bath, comprising in proportion:

|                                                                                              |          |     |
|----------------------------------------------------------------------------------------------|----------|-----|
| Sodium sulphate ( $\text{Na}_2\text{SO}_4$ ) -----                                           | 2 ounces | 100 |
| Sodium chloride ( $\text{NaCl}$ ) -----                                                      | 8 ounces |     |
| Potassium ferrocyanide<br>( $\text{K}_4\text{Fe}(\text{CN})_6 + 3\text{H}_2\text{O}$ ) ----- | 2 ounces |     |
| Water ( $\text{H}_2\text{O}$ ) -----                                                         | 1 gallon |     |

FRED PALMER.  
FRANK PALMER.